

# UNITED STATES PATENT OFFICE.

GERSHOM MOORE PETERS, OF CINCINNATI, AND MILTON FLETCHER LINDSLEY, OF KINGS MILLS, OHIO, ASSIGNEES TO THE KING POWDER COMPANY, OF CINCINNATI, OHIO, A CORPORATION OF OHIO.

## EXPLOSIVE.

988,590.

Specification of Letters Patent.

Patented Apr. 4, 1911.

No Drawing.

Application filed June 6, 1907. Serial No. 377,490.

To all whom it may concern:

Be it known that we, GERSHOM M. PETERS, residing at Cincinnati, county of Hamilton, and State of Ohio, and MILTON F. LINDSLEY, residing at Kings Mills, county of Warren, and State of Ohio, both citizens of the United States, have invented certain new and useful Improvements in Explosives, of which the following is a full, clear, and 10 exact specification.

The invention relates to explosives designed as substitutes for dynamite of approximately 70% to 80% strength. Dynamite, which is the most generally known and used of high explosives, is objectionable in many respects. It freezes at forty-five degrees temperature, and when frozen is not explosive or capable of being detonated, but must be thawed out before using, which is 20 a very troublesome operation, and also very dangerous. Many serious accidents have resulted from the use of dynamite on this account. In hot weather, the nitro-glycerin in the dynamite is liable to exude from the 25 absorbent, which causes great risk and uncertainty in handling it. If dynamite be not properly made and properly neutralized, a condition which is very likely to result because of ignorant or careless employees, 30 decomposition is likely to set in, resulting frequently in most frightful accidents. Then again, a sudden jolt or jar may set off the best dynamite, often without any cause or explanation. All these objectionable 35 features are intensified as the per cents. of strength are increased, so that when dynamite is made to contain a relatively large amount of nitro-glycerin it exudes more readily, is more sensitive, and is much more 40 powerful in its destructive energy.

Dynamite, in its higher per cents. of strength, is also very violent and very shattering and destructive in its effects. It cannot be fired without serious damage and 45 injury to a mine. Often in open air the concussion is such as to endanger life and building, and to be exceedingly annoying because of flying fragments, shocks to the earth and air, and loud reports. Black 50 powder is also objectionable for many reasons. It cannot be used in hard and difficult work as it is not of sufficient strength. In mining operations, when a charge is increased in order to get additional strength,

it not only badly shatters the coal, but 55 throws down the roof, sides and timbers by its concussion. It also produces a great deal of smoke and offensive gas, which interferes with the work going on, and on account of the large amount of flame it generates, it is 60 liable also to set off the natural gas which collects in mines and so produce great destruction of life and property.

It is the object of the invention to furnish an explosive of the highest strength, 65 which shall be safe to handle and transport, which will not freeze, or exude, or spontaneously detonate, will be adapted to do the most difficult work in blasting, which is practically flameless, comparatively noise- 70 less and smokeless, which will not emit injurious and offensive gases, and which will not be objectionable because of the shattering or throwing of fragments, or the causing of disturbances by concussion at points 75 distant from the place of blasting.

The preferred formula contains the following ingredients in substantially the proportions stated:

|                       |     |    |
|-----------------------|-----|----|
| Nitrate of ammonia    | 30% | 80 |
| Nitro-cellulose       | 30% |    |
| Chlorate of potassium | 30% |    |
| Mirbane oil           | 10% |    |

This formula, when the ingredients are 85 of normal strength and quality and properly combined and fired, will produce about three fourths the explosive effect of a like quantity by weight of the commonly termed 75% dynamite.

Nitrate of ammonia, being very rich in 90 gas, is a powerful explosive, as also is nitro-cellulose. Nitro-cellulose is readily sensitive to detonation, besides furnishing the carbon necessary for completing combustion. Chlorate of potassium is both highly explosive and detonative. Mirbane oil is also explosive and detonative, besides furnishing by means of its oily substance, a protection to the other ingredients from the 100 deteriorating effects both of moisture and atmosphere. It also gives a plastic consistency to the explosive when formed in mass, by which it may be more easily handled and packed in cartridges.

The nitro-cellulose is preferably made of 105 wood pulp reduced to dust, nitrated, and thoroughly neutralized and dried. The

nitrate of ammonia and the chlorate of potassium are also thoroughly pulverized and dried. These two ingredients in the proportions substantially as stated are then thrown together in a mixer, such as commonly used for this purpose. The mirbane oil, in substantially the proportion stated, is then poured over these materials in the mixer, after which all are thoroughly mixed or incorporated into a homogeneous substance which is rendered plastic by the aid of the mirbane oil. The mass of explosive thus formed is then packed in cartridges or paper containers, which are thoroughly water-proofed and carefully sealed. It is then ready for use and may be easily detonated by the ordinary primer used in firing dynamite.

This explosive has been found in actual use to be not only very powerful but very safe to handle, is free from danger of explosion by fire, emits little or no flame, smoke or gas, and causes comparatively little report or concussion.

We claim:

25

1. An explosive compound consisting of a thorough intermixture of approximately thirty per cent. of nitrate of ammonia, thirty per cent. of nitro cellulose, thirty per cent. of chlorate of potassium, and ten per cent. of mirbane oil.

2. An explosive compound consisting of an intermixture of nitrate of ammonia, nitro-cellulose and chlorate of potassium in substantially equal proportions, with mirbane oil in sufficient quantity to render the whole plastic.

In testimony whereof we have signed our names to this specification, in the presence of the subscribing witnesses, on this 3d 40 day of June A. D. 1907.

GERSHOM MOORE PETERS.  
MILTON FLETCHER LINDSLEY.

Witnesses:

ELDON R. JAMES,  
A. M. BEEKLEY,  
ED FROHLIGER.

---

Copies of this patent may be obtained for five cents each, by addressing the "Commissioner of Patents,  
Washington, D. C."

---